

Nov. 16, 1926.

1,607,547

F. S. McCULLOUGH

WIRE AND REFRACTORY ARTICLE AND METHOD OF MAKING THE SAME

Filed July 12, 1926

*Fig. 1.*



*Fig. 2.*



*Fig. 3.*



INVENTOR

Frederick S. McCullough  
by his attorneys  
Byrnes, Stebbins & Kambe

## UNITED STATES PATENT OFFICE.

FREDERICK S. McCULLOUGH, OF EDGEWOOD, PENNSYLVANIA.

## WIRE AND REFRACORY ARTICLE AND METHOD OF MAKING THE SAME.

Application filed July 12, 1926. Serial No. 121,852.

This invention relates to the manufacture of wire and porcelain or like refractory articles, and constitutes an improvement on the invention disclosed in my Patent No. 1,549,591 dated August 11, 1925.

In the manufacture of certain types of electrical devices wherein a heating wire is passed through a body of refractory material, such for instance as a porcelain body, 10 it has been found that the wire, which is usually of a small diameter, has a relatively short life when it is heated and cooled in its subsequent use.

Various attempts have been made to remedy this difficulty, one method being disclosed in my co-pending application Serial No. 79,351 filed January 5, 1926. In my said co-pending application, I have disclosed a method wherein the porcelain or other refractory material is applied under such conditions that the wire is firmly held in the porcelain, and the porcelain is in effect shrunk onto the wire.

I have now discovered that the length of 25 life of the wire may be very materially increased if the wire does not fit too snugly in the porcelain, so that it may be free to expand and contract therein without undue chafing against the body of the refractory.

30 The nature of the present invention may be readily understood by reference to the accompanying drawing, wherein:

Figure 1 is a diagrammatic view illustrating a wire and porcelain article mounted in 35 a vessel which may be evacuated, and wherein the porcelain or other refractory may be fired.

Figure 2 is an enlarged detail section of a portion of the wire and porcelain article before it has been fired.

Figure 3 is a transverse section in the plane of line III—III of Figure 2.

The article includes a rod 5 of porcelain or other refractory or other suitable refractory which has one or more holes 6 therethrough, through each of which is passed an electric resistance wire 7. Surrounding the porcelain is a metal shell 8, which is preferably in the form of a complete metal cylinder, and it is preferably of a magnetic material, such as nickel. This article may be supported by a base or other supporting means 9. The article after it has been assembled, and before the porcelain has been entirely fired, is placed within a vessel of glass or other suitable material, such vessel

being designated 10, and this vessel may be sealed to the support 9, or otherwise fitted thereto, in such manner as to form an airtight joint. Leading from the vessel is a tube 11, which is connected to a vacuum pump or other suitable exhausting means, not shown.

Surrounding the vessel are several convolutions of wire which may be included in a high frequency, or radio frequency, circuit. When the coil 12, comprised of the convolutions of wire, is energized, the inductive field thereof effects a heating of the metal shell 8, raising the temperature of the porcelain body 5 to a point sufficient to heat treat the porcelain and drive out the occluded gases.

The porcelain, when it is thus heat treated under reduced pressure, tends to contract, so that the holes therein have a tendency to become smaller. According to the present invention, it is proposed to make the holes at least one and one-half times as large as the diameter of the wires 7. This will permit the hole to shrink without the porcelain being forced into intimate contact with the wires, so that while the wires are supported by the body of the refractory, they are sufficiently free to expand and contract in their subsequent use without binding and without such strain or chafing as will result in the disintegration and pulling apart of the heater wire. This insures a long life for the heater or other device constructed in this manner.

The hole is preferably made no larger than substantially one and one-half times the diameter of the wire 7, because if it is made larger, the wire does not receive proper support in the porcelain after the porcelain or other refractory has been heat treated and the heat of the wire is not so effectively transmitted to the body of the refractory, so that the efficiency of the device as a heater for certain purposes is not as great as it should be. I do not confine myself to this particular ratio between the wire and the raw refractory, as the hole may be made somewhat greater or less, according to the character of the refractory and the extent of contact desired between the porcelain and wire in the finished article.

A particular advantage of the present invention resides in the construction of a heater wherein the heater wire may be embedded in a mass of porcelain or other refractory and wherein the embedded heater

wire is not subject to undue binding or chafing sufficient to result in its disintegration, but wherein the wire is fairly well supported in the porcelain or other refractory, and wherein heat may be effectively conducted from the wire through the refractory.

While I have illustrated a preferred manner of firing the porcelain in a vacuum, it will be understood that I do not limit myself to the particular method therein disclosed, nor to the use of radio frequency currents as a means for heating the wire and porcelain article, and it will be understood that various changes and modifications may be made in the construction of the article and the method of effecting the invention within the spirit of my invention and under the scope of the appended claims.

20 I claim as my invention:

1. The herein described method of manufacturing a wire and porcelain article, which consists in passing the wire through a hole in the porcelain which is substantially larger than the diameter of the wire, and then heat treating the porcelain.

2. The herein described method of forming a wire and porcelain article which consists in passing a wire through a hole in a porcelain rod wherein the diameter of the hole is substantially one and one-half times

the diameter of the wire, and then heat treating the porcelain in a vacuum.

3. The herein described method of forming a wire and porcelain article which consists in passing a wire through a hole in a porcelain rod wherein the diameter of the hole is substantially one and one-half times the diameter of the wire, and then heat treating the porcelain under a reduced pressure.

4. The herein described method of forming a wire and porcelain article, which consists in passing the wire through a hole in a refractory rod wherein the diameter of the hole is larger than the diameter of the wire so that the wire is loose therein, applying a metal shell to the outside of the porcelain, and then heating the porcelain rod and shell in a vacuum by induction to heat treat the porcelain and contract the porcelain about the wire.

5. A wire and porcelain article of the type described comprising a porcelain rod having a hole therethrough and having a wire passed through the hole wherein the wire is loosely received in the hole but is supported by the porcelain.

In testimony whereof I have hereunto set my hand.

FREDERICK S. McCULLOUGH.